

# United States Patent Office

3,164,448

Patented Jan. 5, 1965

1

3,164,448

## PREPARATION OF METALLIC SURFACES FOR CLADDING WITH COMMINUTED METALS AND THE PRODUCTS SO CLAD

Rolfe Pottberg, Baltimore, Md., assignor to Peen Plate, Inc., Baltimore, Md., a corporation of Maryland  
No Drawing. Filed Nov. 15, 1960, Ser. No. 69,297  
13 Claims. (Cl. 29—194)

This invention relates to the preparation of metallic surfaces for the application of coatings of other metals where these are applied in solid, comminuted form to the prepared surface and products so coated.

This application is a continuation in part of my pending application Serial No. 388,702, filed October 27, 1953.

In application, Serial No. 388,702, it was shown that thin films of copper applied by simple immersion treatments served greatly to facilitate the deposition and adhesion of metal coatings originally supplied in the form of finely divided solid powder particles, usually in liquid environments such as those described in U.S. Patent 2,640,002 and British Patent 534,888, and under conditions tending to densify and consolidate layers of such particles into a dense, adherent film, usually by subjecting to agitation and impact in the presence of a surrounding, suspending mass of suitable impacting particles.

It has since been found that the mechanism presumed effective in the former case, i.e., metallurgical compatibility or relative "ease of wetting" of one metal by another, or mutual solid solubility, is not the only mechanism responsible for the effectiveness of such films as a preliminary surface treatment for such method of metal cladding; but that another and in some cases more important mechanism is operative. This in turn has led to the discovery of other such preliminary metal films, some of which are effective to an even greater degree than described for instance in Serial No. 388,702. This contributing factor, found to be effective in the original case referred to as well as in the newly discovered instances is related to the solution potential of the metal of the preliminary film relative to that of the metal of the powder particles to be applied to said film. There is an important correlation and proportionality between solution potential differences and deposition efficiencies in whatever liquid solutions are used; if the solution potential of the base metal surface is lower than that of the metal powder particles. Other metals which may be applied by immersion means are also effective, some of them to an even greater degree than others and, in many instances, certain metals having the immersion coating thereon will be receptive to the metal particles which without the immersion coating will not be receptive to the metal particles.

An object of the present invention is to so prepare a metallic surface by applying thereto a thin adherent coating of another metal having the unique property of causing finely divided particles of a third metal to be attracted and adhered thereto in preparation for later steps to further coalesce and densify the particles.

Another object of the invention is to prepare the surface of the base metal by applying a thin immersion coating of a metal thereto having a lower solution potential than the base metal and then applying finely divided particles of a metal having a higher solution potential than the immersion coating, to which immersion coating the particles will be caused to be attracted and adhered in preparation for whatever steps are taken simultaneously or later to consolidate or densify the coating of the particles.

Another object of the invention is to overcome any unevenness of the surface characteristics of the base metal by the immersion coating, which produces an even coating over the base metal and changes the characteristics

2

thereof whereby they are substantially the same point to point; thus giving the advantage that the surface of the thus coated base metal is metallurgically uniform and the metal particles subsequently applied thereto accumulate and adhere with greater uniformity.

A still further object of the invention is to provide a coated object which, in addition to being more uniform, is superior in corrosion resistance by virtue not only of added coating uniformity but which is also quantitatively superior in the sense of having a thicker coating as a result of the particular processing, as well as a coating which is qualitatively superior due not only to superior adhesion but also to favorable galvanic effects arising from the imposition of the thin, more noble metal film between the less noble base metal and metal cladding surrounding it.

It has been found by actual tests and examples herein-after recited that when a piece of a base metal or an article of a base metal has applied thereto a thin coating of a metal having a lower solution potential than that of the metal particles to be applied and that when the thus coated base metal is placed in agitated relationship to a slurry containing the metal particles in usually an acid or an acid salt solution, the metallic particles will tend to be attracted to the coated surface of the metallic article and will be caused to accumulate upon and adhere to the coated surface and also to each other with tenacity so that the thus adhered particle layer or bed is highly resistant to removal by mechanical or hydraulic influences encountered in the course of further processing, to consolidate and densify the final coating.

Impacting media may be added to the slurry consisting of the appropriate salts in solution, the metallic particles and the immersion coated metallic articles; and the whole agitated together such as in a tumbling mill, the same being rotated for a predetermined period of time so as to finally compact the particles against each other and the surface of the immersion coating. By "impacting media" is meant a matrix material consisting of a mass of discrete solid granules usually much smaller than the articles or objects but much larger than the metal of the powder particles, inert to the particular chemical environments employed and serving the purpose of separating and suspending the objects from one another in the course of mechanical agitation, as well as to supply a multiplicity of randomly distributed impacts to the surfaces being so coated. Such granules may be spherical or irregular, and be metallic, ceramic, mineral, vitreous or even consist of the objects themselves if these are small and numerous enough.

However, when placed in an agitated slurry, the metallic articles are found to be relatively adherently coated with undistorted particles of the metal coating powder in the absence of any impacting or other forces sufficient to affect final consolidation of the coating.

The preliminary, immersion or substrate coating referred to herein defines the thin coating which is applied directly to the metallic object and to which subsequently is applied a coating of the metal powder particles.

I use as an immersion coating salts of the following metals: cadmium, tin, lead, silver, copper and mercury.

The metal particles to be applied to the immersion coating are selected from the group: zinc, cadmium, tin, lead, nickel, copper and silver and alloys thereof, in general, zinc and cadmium behave similarly, as do brass and copper.

The invention in one of its aspects, involves the process of treating the base metal to be coated in ionized solutions of salts of metals having a lower solution potential than the metal of the base. Since the suitable metals can usually be easily deposited by well-known, immersion means on the most commonly encountered, i.e., ferrous

surfaces, I utilize a salt of a metal which has a lower solution potential than the metal of the base. It is usually not necessary to resort to electrolytic means for the deposition of the lower metals. In general, the lower the solution potential of the suitable metals recited the more readily the immersion coating is adhered to the surface of the base metal. For reasons recited in the original application and which apply equally as well in this application, copper is and remains a logical, highly effective and economical choice as the metal of the immersion coating; particularly where metals such as zinc and cadmium are to be deposited on ferrous basemetals.

Procedures for applying immersion films of the preliminary coating metals recited are well-known to the art and appear in standard reference texts available to the metal plating trades, for instances, as disclosed in, and may be considered as part hereof, the publication published by Finishing Publications, Inc. entitled "Metal Finishing Guidebook Directory." Improved proprietary formulations and materials are also available.

The metal article may have various surface unevennesses, such as unevenness in its metallurgical characteristics, which characteristics may have been formed during the molding or working or heat treatment of the article. The present invention overcomes unevennesses from point to point on the surfaces; both of metallurgical characteristics and of relative solution potential; such as to affect the evenness with which the particle layer accumulates. The immersion coating itself has the same characteristics from point to point, thus making a uniform surface on which the particles are subsequently uniformly accumulated. The immersion coating so masks the metallic article that the particles being applied thereto are not affected by the base metal but are only affected by the immersion coating.

The thus coated articles are placed in a slurry, which slurry will contain the metallic particles in a, preferably acid, salt solution with or without an impacting medium. Thus slurry, together with the coated metallic articles may then be placed, for example, in a tumbling drum and the same rotated for a predetermined period of time. When the metallic articles are removed from the drum, it will be found that they have adhered to their surface practically all of the metallic particles. Especially if an impacting media is used in the drum and when the articles are removed therefrom, the metallic particles will be found to have been compacted and densified on the article and the article is now ready for the use to which it is to be put without further treatment. The type of coating which results when the final coating has been densified in the foregoing manner may generally be described as follows, following metallographic sectioning and chemical treatment:

A very thin, crystalline deposit of the lower solution potential metal deposit fills microscopic pores and cavities in the base metal and can be seen to be sandwiched between the latter and a much thicker coating comprised of the original metal powder particles. A section of this final coating in turn, after appropriate chemical etching, can be seen to consist of the particles of the original coating metal perceptibly distorted in such a manner as usually substantially to eliminate all interstitial voids and in some cases to establish a metallurgical bond between the particle interfaces. This distortion is in a horizontal plane parallel to the surface to which the coating is applied and may vary from such distortion as is necessary simply to substantially eliminate all interstitial voids between such original particles, to a point at which the particles are extremely distorted in a horizontal dimension with corresponding reduction in vertical dimension; resulting in a lamellar or stratified appearance. A further and often distinguishing characteristic of the particular type of coating which results, following resort to the herein set forth expedients, is that traces of the metal of the immersion coating can be metallographically dis-

cerned between particles of the final coating metal adjacent to the interface of the two coatings and at some distance from the original surface. These traces may be in the form of discrete occlusions of the original immersion coating metal between particles of the cladding metal or they may be diffused therewith; such diffusion being most readily discernible under polarized light. It has been surmised that this may result from some of the metal of the immersion film having gone into solution during the particle coating operation and reprecipitating out on the metal of the particles; possibly tending to assist in preliminarily securing the particles in position.

When no impacting media is used in the slurry and even with only slight agitation, the metal particles appear to have a strong physical affinity for the substrate coating and a stronger affinity for one another than is the case in the absence of the favorable substrate coatings claimed herein. Further, there is evidence to indicate that the substrate coating attracts the metal particles to the surface prior to actual physical contact therewith, and the particles are sufficiently strongly adhered to the substrate coatings and to each other that they strongly resist removal by the mechanical and hydraulic forces encountered in the course of the plating operation. Additionally, such tenacious, initial adherence makes less critical the choice of mechanical conditions necessary to avoid chipping off of the coating at sharp edges prior to the time that a final coating has been fully metallurgically integrated and adhered.

It is sometimes desirable to apply an intermediate immersion coating, in cases where the solution potential of the immersion coating desired is so much lower than that of the metal of the article itself that spongy and poorly adherent immersion coatings result, unless an immersion coating of intermediate solution potential is interposed. The use of copper prior to application of silver or mercury is an example.

As an example in which differently treated surfaces have metallic particles applied thereto under otherwise identical conditions, but in physical separate apparatus, the following test was made:

Four pound batches of 1" diameter by  $\frac{1}{16}$ " hot rolled steel washers were used in which all were preliminarily thoroughly cleaned and all but one batch immersion coated with tin, lead, copper, silver and mercury respectively. The slurry in each case consisted of six pounds of 12 mesh fused aluminum oxide granules, 170 grams of fine, high purity condensed zinc dust and approximately 600 cc.'s of water acidified with 35 grams of zinc chloride. (In the one batch having an immersion coating of silver thereon, an equivalent amount of hydrofluoric acid was used). Each batch was agitated in a small, approximately 4000 cc.'s tumbling mill for two hours at ambient temperature. After the treatment the washers were removed from each batch and washed and the thickness of the zinc was measured on each and found to be as follows:

| Surface:                  | Thickness of zinc deposited inches |
|---------------------------|------------------------------------|
| Clean steel               | .0001                              |
| Immersion applied tin     | .00025                             |
| Immersion applied lead    | .0016                              |
| Immersion applied copper  | .0006                              |
| Immersion applied silver  | .004                               |
| Immersion applied mercury | .006                               |

Such coating thicknesses are found to generally reflect the different solution potential with respect to zinc in the particular electrolyte or acid or acid salt employed.

In another example, similar objects with dissimilar metal surfacing were plated together at the time in the same apparatus. Two lbs. of  $1\frac{1}{4}$ " by 11 gauge iron roofing nails were divided into four equal half pound quantities. One was merely acid cleaned, and each of the three remaining half pound quantities received immersion coatings respectively of copper, silver and mercury. (For reasons

previously stated the latter two immersion coatings were superimposed upon intermediate immersion coatings of copper. Such immersion films deposited under normal conditions are extremely thin by comparison with discernible thicknesses recited herein and the extent to which their thickness contributes to that of the final film can be disregarded.) The two pounds of nails were placed in a tumbling mill together with six of glass beads of sizes ranging between minus 25 mesh to plus 100 mesh, 85 grams of zinc dust and 600 cc.'s of water acidified with seven cc.'s of 180° sulphuric acid. The drum was rotated for 1½ hours and at the completion thereof the articles were observed to have the following amounts of plating thereon:

| Surface:          | Thickness of zinc deposited inches |
|-------------------|------------------------------------|
| Clean iron        | .0000                              |
| Immersion copper  | .0015                              |
| Immersion silver  | .0047                              |
| Immersion mercury | .008                               |

<sup>1</sup> No plate.

In a further example in similar equipment two separate, two pound batches of such 1" washers were processed under otherwise identical conditions using minus 395 mesh brass powder, glass beads and a dilute citric acid solution. Half the quantities of washers in each test were merely cleaned and the other half surfaced respectively with immersion coatings of mercury and silver. The results in the two tests showed a continuous brass coating for the immersion surfaced washers and a discontinuous coating of the unsurfaced washers with a majority of the area of the same uncoated.

In a similar series of tests two pound batches of small iron powder metallurgy parts were separately processed for 2 hours in the presence of 9 pounds of brass coated steel impacting particles approximately  $\frac{1}{16}$ " in diameter, and 30 grams of minus 395 mesh atomized brass powder. Previously lead surfaced articles had the heaviest coating, unsurfaced clean steel objects had coatings which while substantially continuous were only approximately 1 powder particle thick, and in the third and fourth tests previously tin and zinc coated objects received no coating. (In the latter two cases the tin and zinc were mechanically applied.)

In another test one inch clean steel washers were placed in one drum and a similar amount, which were immersion coated with mercury, in another, each drum receiving six pounds of 12 mesh synthetic alumina granules, 1% citric acid and 100 grams minus 395 mesh brass powder. After 1 hour the initially unsurfaced steel washers had a film of brass so light as to be characterizable only as a color whereas the mercury coated washers had .0008" of brass thereon.

If copper powder is substituted for brass powder proportionate results are observed except that copper deposits with somewhat greater efficiency from similar solutions. The efficiency of the deposition of both copper and brass appears to be improved if sulphuric or phosphoric acid is substituted for the citric acid in those examples mentioned above.

In the depositing of nickel on steel, two tests were made using clean steel objects in one test and steel objects having an immersion coating of lead thereon. The slurry contained fine nickel powder, citric acid and small glass beads approximately three times the weight of the objects. The unsurfaced steel objects received a coating which could not be measured even by electromagnetic means but those immersion coated with lead received an apparently continuous coating of nickel.

To indicate the extent to which the particles tend to adhere to one another and to the base prior to, or in the absence of more drastic means of effecting their final consolidation into an integrated coating the following test was made. A small quantity of small nails was used

in the presence of a relatively large volume of soft polyethylene granules, to minimize the possibility of inter-object impact contributing to coating densification, and to largely remove the possibility of impacting the coating other than with material much softer than that of the metal itself. In this case dilute 1% citric acid solution was used with approximately 3000 cc.'s of  $\frac{1}{8}$ " diameter polyethylene granules and 30 grams of condensed zinc dust in 4000 cc. equipment. In spite of the fact that test conditions were established to minimize impact and attrition adequate to affect the plastic deformation or swaging of the metal of the powder particles, it was observed that a hard, thick, relatively adherent (although almost completely unpolished) coating resulted.

It has been shown herein that the particles will adhere to metallic articles previously surfaced with herein recited coatings within a relatively short time. It has been further shown that objects with an immersion coating of copper, for example, agitated in the presence of slurries of fine glass beads and zinc dust in the appropriate solutions may accumulate on their surfaces the majority of all the dust present in their vicinity within a space of a few minutes; the dust being distributed uniformly over the surfaces of the objects and being, naturally, sufficiently adherent to have resisted the forces of attrition, mechanical and hydraulic, inherent in the conditions of operation. Under these conditions the zinc dust is not naturally perceptibly affected and still resembles the original zinc dust in appearance. In such instances the matrix of impacting particles have served simply to uniformly disperse and separate both objects and zinc dust particles and provided no significant mechanical action. Such coatings even in this condition are sufficiently dense and they have a limited usefulness after drying the same at moderate temperatures.

Thus it will be seen from the examples that metal surfaces having a coating referred to herein of metal having a lower solution potential than the metal of the surface, and deposited from ionized solution, can be coated with layers of metallic powder particles of a metal having a higher solution potential than that of the coating, and that the resulting such coating layer of particles is intrinsically more strongly adherent to such coated metal surface, prior to or in the absence of other means to further densify and consolidate such overlayer of particles. Further, it has been shown that more than one means may be used to finally prepare such overlayer of powder particle for final usefulness. It has also been further shown that the majority of the metal powder particles are attracted and will adhere to the immersion coated article within a relatively short time, sufficiently strongly to resist removal under sometimes drastic conditions of mechanical and hydraulic scrubbing.

I claim:

1. In a process for cladding metal article surfaces with adhered, compacted multilayers of interfitting, solid and discrete mechanically distorted particles of another metal by immersing said surfaces in dynamically agitated, hydraulic suspensions of said metal particles in aqueous electrolytes, the step of preliminarily applying directly onto said surfaces a relatively thin layer of a third metal having a lower solution potential than the metal of the metal powder particles.

2. The process for cladding metal article surfaces as set forth in claim 1 wherein the preliminarily applied coating metal has a lower solution potential than that of the metal article surfaces and is applied to said metal article surfaces by immersing the metal article in a solution of salts of said preliminarily applied third metal.

3. The method as set forth in claim 1 in which the preliminarily applied coating is selected from the class of metals consisting of cadmium, tin, lead, copper, silver and mercury.

4. The method as set forth in claim 1 in which the solid particles are selected from the group of metals consisting

of zinc, cadmium, tin, copper, lead, nickel, silver and the alloys thereof.

5. In a process for cladding metal article surfaces with adhered, compacted multilayers of interfitting, solid and discrete mechanically distorted particles of another metal by immersing said surfaces in dynamically agitated, hydraulic suspensions of said metal particles in acidified solutions, the step of preliminarily applying directly onto said surface a relatively thin layer of a third metal having a lower solution potential than the metal of the metal powder particles.

6. An article having a base metal surface and a permanent metallic coating thereon, the coating consisting essentially of:

a relatively thin, ionized salt solution deposited crystalline coat of a first metal adhering directly to the base metal surface; and

a relatively thick coat of built up layers of mechanically distorted and closely interfitting discrete and distinct powder particles of a second and different metal superimposed directly on the first coat, the second metal having a solution potential higher than the solution potential of the first metal.

7. An article according to claim 6 wherein the base metal surface is of a solution potential higher than the solution potential of the first metal.

8. An article according to claim 6 wherein the first metal is selected from the group consisting of cadmium, tin, lead, copper, silver and mercury; and the second and different metal is selected from the group consisting of zinc, cadmium, tin, nickel, copper, lead, silver, and alloys thereof.

9. An article according to claim 8 wherein the base metal surface is ferrous.

10. An article according to claim 6 wherein the base metal surface is ferrous, the first metal is copper, and the second metal is zinc.

11. A method of coating metal surfaced articles comprising the steps of:

immersing the metal surfaced articles in an ionized acidic salt solution of a first metal having a solution potential lower than the solution potential of the metal surfaced articles to deposit a relatively thin crystalline layer of the first metal onto the metal surfaced articles, and then

10 impacting the immersion deposited articles with a dynamically agitated hydraulic suspension of powder particles of a second metal in a plate promoting liquid carrier to further coat the articles with a superimposed coating of multi-layers of impacted and mechanically distorted, work hardened discrete and distinct interfitting particles, the second metal being different from the first metal and having a solution potential higher than the solution potential of the first metal.

12. The method according to claim 11 wherein the first metal is selected from the group comprising of cadmium, tin, lead, copper, silver and mercury; and the second metal is selected from the group consisting of zinc, cadmium, tin, nickel, copper, lead, silver and alloys thereof.

13. The method according to claim 12 wherein the metal surfaced articles are ferrous.

References Cited in the file of this patent

UNITED STATES PATENTS

|           |              |       |                |
|-----------|--------------|-------|----------------|
| 2,251,410 | Koehring     | ----- | Aug. 5, 1941   |
| 2,428,033 | Nachtman     | ----- | Sept. 30, 1947 |
| 2,459,172 | Luketmeyer   | ----- | Jan. 18, 1949  |
| 2,473,712 | Kinney       | ----- | June 21, 1949  |
| 2,640,002 | Clayton      | ----- | May 26, 1953   |
| 2,667,429 | Diffenderfer | ----- | Jan. 26, 1954  |
| 2,873,216 | Schnable     | ----- | Feb. 10, 1959  |
| 2,892,801 | Sargent      | ----- | June 30, 1959  |
| 2,902,748 | Schaefer     | ----- | Sept. 8, 1959  |
| 2,916,337 | Fike         | ----- | Dec. 8, 1959   |